

# UNITED STATES PATENT OFFICE.

JOHN N. LUTZ, OF PORTSMOUTH, OHIO.

## PHOTOTYPOGRAPHY.

SPECIFICATION forming part of Letters Patent No. 240,262, dated April 19, 1881.

Application filed January 11, 1881. (No specimens.)

*To all whom it may concern:*

Be it known that I, JOHN N. LUTZ, a citizen of the United States, residing at Portsmouth, in the county of Scioto and State of Ohio, 5 have invented certain new and useful Improvements in Phototypography; and I do hereby declare the following to be a full, clear, and exact description of the invention, such as will enable others skilled in the art to which it app- 10 pertains to make and use the same.

This invention relates to improvements in the art of producing photographic pictures upon wood, especially such as are to assist engravers. The preparation of the wood for this 15 purpose has been hitherto accomplished by processes both expensive and tedious, and the purpose of this invention is to avoid the difficulties heretofore met with and provide a process whereby a photographic picture of a very 20 superior character can be obtained at a merely nominal price.

A block of wood of proper quality and proper size is first coated with white water-color and water, which are rubbed over the wood until 25 a white and perfectly smooth surface is produced, and the excess is then removed. After the wood has been whitened and smoothed it is then treated with the following solution: I take five grains of citric acid, five grains of 30 chloride of ammonium, and twelve grains of gelatine, and dissolve and thoroughly mix them in one ounce of water. The solution is heated, and it is then poured over the surface of the block. It is left on the block from three to five 35 minutes, and the block is then allowed to dry.

One great advantage incident to the above solution is that it can be kept for a long time, and can therefore be prepared in large quantities and can be put upon the market as a 40 manufacture.

After the block is dry it is treated with the following preparation: Nitrate of silver is dissolved in water in the proportion of forty grains of the former to one ounce of the latter.

45 The solution is then filtered through paper, and the block is treated with it in a manner similar to that described above. After the block has been subjected to the action of the

latter solution for two or three minutes it is dried in the dark, as the block is now sensitive 50 to light. After it is dry it is treated for about ten minutes with ammonia, and it is then ready to receive the impression from the negative. After the impression has been taken and the negative removed the block is washed 55 and subjected to a hypo-bath for about five minutes, after which it is again washed, and is then ready for the engraver.

The most important part of my process is that comprised in the second step, or the application of chloride of ammonium, gelatine, water, and citric acid, &c. By means of this preparation I obtain a much clearer impression than can be procured by the ordinary agents. It keeps the silver from sinking while 65 the light is acting through the negative. It also gives a vigor and brilliancy to the picture, producing very clear white in the lighter portion and deep black in the shadow.

I do not wish to be understood as claiming, 70 broadly, the use of citric acid alone as an ingredient in preparations for photographing upon wood for engraving, as I am aware that various acids have been heretofore used for this purpose; but I believe myself to be the 75 first to have employed the hereinbefore-described preparations in the exact manner and in the sequence which has been set forth.

What I claim is—

The herein-described process for preparing 80 wood to receive a photographic impression for engraving, which consists in first applying to the surface of the wood an enameling or whitening preparation, then a preparation consisting of chloride of ammonium, citric acid, gelatine, and water, in substantially the proportions specified, then a silver sensitizing preparation, and finally ammonia, substantially in the manner and for the purposes set forth.

In testimony whereof I affix my signature 90 in presence of two witnesses.

JOHN N. LUTZ.

Witnesses:

I. N. ZOELLNER,  
C. A. ZOELLNER.